

Jan. 6, 1925.

1,522,291

G. W. ELMEN

LOADED SIGNALING CONDUCTOR

Filed Dec. 28, 1920



Inventor:  
Gustaf W. Elmen.  
by Jas. C. Palmer  
ATTY.

## UNITED STATES PATENT OFFICE.

GUSTAF W. ELMEN, OF LEONIA, NEW JERSEY, ASSIGNOR TO WESTERN ELECTRIC COMPANY, INCORPORATED, OF NEW YORK, N. Y., A CORPORATION OF NEW YORK.

## LOADED SIGNALING CONDUCTOR.

Application filed December 28, 1920. Serial No. 433,696.

To all whom it may concern:

Be it known that I, GUSTAF W. ELMEN, a citizen of the United States, residing at Leonia, in the county of Bergen, State of New Jersey, have invented certain new and useful Improvements in Loaded Signaling Conductors, of which the following is a full, clear, concise, and exact description.

This invention relates to loaded signaling conductors such as are used for instance in submarine cable signaling.

There are two generally recognized methods of loading signaling conductors. Perhaps the more extensively used method is that of inserting so-called loading coils at intervals in the circuit. The other method is generally called continuous loading. In either method of loading the object is the same, namely, to introduce an amount of inductance per unit length which will satisfy the condition of approximately distortionless transmission of an alternating or pulsating electric current.

Both in the case of loading coils and in the case of continuously loaded conductors, the electrical characteristics which it is desirable to have in the magnetic material used for loading are the same. These characteristics are high specific resistance to keep down the eddy currents in the loading material, extremely low hysteresis loss, magnetic stability or constancy in permeability as regards talking currents even though large currents are superposed on the circuit, and as high permeability at low magnetizing forces as is consistent with the foregoing characteristics.

The use of tape or wire, heretofore used for continuous loading, is not without its disadvantages. It has been found in this connection that if the loading material be applied in such a way as to grip the conductor too tightly, the resulting strain greatly reduces the permeability of the loading material. If, on the other hand, the loading material be applied so loosely as to leave even small interstices between the successive windings, pressure, especially in the case of submarine cables, tends to force the insulating covering between the conducting core and the loading material, thus impairing the efficiency of the cable. In any case, it has proven impossible to prevent the introduction of air gaps between the successive windings, and hence,

a reduction in the effective inductance has resulted.

It is one object of this invention to provide a method of producing a continuously loaded signaling conductor in which the metal core adapted to conduct the signaling currents is surrounded by a sheathing of a magnetic alloy adapted to serve as a loading material.

Another object is to provide a structure of this type in which the loading material cannot be separated from the conductor by forces to which it may be subjected in use.

Another object of the invention is to provide a continuously loaded signaling conductor of which the overall diameter is constant.

In the following description reference is made to Fig. 1 which shows diagrammatically one means of practicing the invention and Fig. 2 which shows a section of a cable comprising conductors loaded according to the invention.

It has been found that the high permeability of iron-nickel alloys in which a large percentage of nickel is present, renders them particularly suitable as a loading material for signaling conductors. In a copending application of Gustaf W. Elmen, Serial No. 473,877, there is fully described the advantages of these alloys as loading material and the method of applying them to a signaling conductor in the form of a spirally laid wire or tape.

Attempts have been made in the past to utilize an alloy of iron and a small percentage of nickel as a loading material for signaling conductors by electroplating the alloy upon the conductor. It is now known, however, that a deposit of alloy cannot be obtained by this method. Instead, a mixture of iron and nickel is deposited out, each metal retaining its individuality. Moreover, the addition of a small amount of nickel to iron, even if an alloy were produced, is less desirable as a loading material for telegraph and telephone wires, than pure iron. But when the content of nickel is sufficiently increased, the alloy has such high permeability for low magnetizing forces of the order used in signaling, such low hysteresis loss and high resistivity that it becomes peculiarly well fitted to this purpose.

This invention is based on the discov-

ery that when nickel and iron are electro-deposited on a conducting wire in the form of a coating of the two metals in which a large percentage of nickel is present, and 5 the deposit is heated to a temperature below the melting point of copper, which is well below the melting points of either nickel or iron, this temperature is high enough to produce an alloy of the iron 10 and nickel which will have the properties desired for loading a telegraph or telephone conductor.

In accordance with the preferred method of carrying out the invention a coating of 15 iron and nickel is electrolytically deposited upon the copper conductor, the deposit containing at least 20% of nickel, and the deposit of iron and nickel is subsequently heated to a degree below the melting point 20 of the copper conductor. By this treatment a sheathing of high permeability is obtained. It may be desirable to pass the loaded conductor through a die in order to produce a smooth surface in the event 25 that the alloying process has left a rough exterior. Any well known suitable method of obtaining a deposit electrolytically and any suitable type of furnace for heating the conductor may be utilized. One suitable 30 form of apparatus is disclosed in Fig. 1, which illustrates a conductor 3 being passed slowly through an electrolytic bath 4 of which it forms the cathode. The conductor is connected to a source of current 5 by means of a roller contact 6. The anode 35 7, which is also connected to source of current 5, is composed of nickel and iron in the proportions desired. The conductors are then passed through a furnace 8 or 40 are otherwise heated to alloy the nickel and iron. Coils of wire may, of course, be used as a cathode and thereafter removed from the bath and heated in the furnace. Fig. 2 is self-explanatory. It 45 shows a cable made up of a plurality of copper wires loaded in accordance with the invention. In the case of long submarine cables a single conductor would ordinarily be employed.

50 A loaded signaling conductor produced

in accordance with the method herein described has a uniform diameter throughout its length, the distance from the center of the core to the circumference of the loading sheath being everywhere equal. An 55 important advantage of this form of loading is that the permeability of the layer of loading material does not change if the loaded conductor is subjected to great pressure, as is the case with submarine cables 60 laid in considerable depths of water. Moreover, there is no tendency of the layer of loading material to become separated from the conductor so as to permit insulating material to be forced into the intervening 65 spaces and thus destroy the symmetry of the cable structure.

What is claimed is:

1. The method of producing a continuously loaded signaling conductor which comprises plating a coating of iron and nickel upon the surface of the conductor, the nickel comprising not less than 20% of the deposit, and subsequently heating the deposit to a temperature well below 70 the melting point of either nickel or iron and in the region of the melting point of copper to obtain an alloy of the iron and nickel having high permeability for magnetizing forces of the order used in signaling. 75

2. The method of continuously loading a copper signaling conductor which comprises electroplating a coating of iron and nickel upon the surface of the copper, the nickel constituting at least 20% of the deposit, and subsequently heating the deposit to a temperature below the fusing point of copper to alloy the iron and nickel. 85

3. A continuously loaded signaling conductor comprising wire of material of high conductivity having electroplated thereon a coating of alloy comprising nickel and iron, the nickel forming at least 20% of the alloy. 90

In witness whereof, I hereunto subscribe my name this 22nd day of December A. D., 1920.

GUSTAF W. ELMEN.